

C. W. ROYCE.

FABRIC.

APPLICATION FILED MAY 29, 1915.

1,163,262.

Patented Dec. 7, 1915.



WITNESSES.

Ada C. Fagerly

Grace A. Davis.

INVENTOR.

Charles W. Royce  
Joseph A. Miller  
ATTORNEY.

# UNITED STATES PATENT OFFICE.

CHARLES W. ROYCE, OF PROVIDENCE, RHODE ISLAND, ASSIGNOR, BY MESNE ASSIGNMENTS, TO CUSHION FABRIC COMPANY, OF PROVIDENCE, RHODE ISLAND, A CORPORATION OF RHODE ISLAND.

## FABRIC.

1,163,262.

Specification of Letters Patent.

Patented Dec. 7, 1915.

Application filed May 29, 1915. Serial No. 31,232.

To all whom it may concern:

Be it known that I, CHARLES W. ROYCE, a citizen of the United States, residing at Providence, in the county of Providence and State of Rhode Island, have invented a new and useful Improvement in Fabrics, of which the following is a specification.

The invention relates to certain new and useful improvements in fabric known commonly in the trade as composition leather fabric.

It has for its primary object to provide an efficient substitute for leather and the uses of leather in connection with textile machinery and is particularly adaptable to combers, aprons or belts and for roll coverings.

The invention consists essentially in a fabric having a coating of oil capable of being oxidized to produce a firm but flexible surface attached thereto.

The drawing is only illustrative in the sense that the materials of the various layers or coatings are understood to be intimately united with each other by proper mixing.

The fabric is preferably formed by napping the surface of a woven wool, cotton, or wool and cotton fabric so as to produce a fabric of springy or resilient character and the preferred fabric is one having a cotton base and a wool nap. To the napped wool surface of the preferred fabric is applied a series of coatings of a compound of oxidizable oil, as linseed oil or its equivalent, fine clay, and a pigment as lamp black. Any of the well-known coloring pigments may be used to give desired appearance. The clay is added in a sufficient quantity to give the compound a paste-like consistency.

In practice the coating is applied to the napped side of the fabric each coating being dried by passing the fabric through a drying machine.

To the composition of the coatings ap-

plied subsequent to the first application may be added manganese, umber, or other substances for the purpose of improving the toughness of mixture and adding life to the fabric. After a suitable number of coatings have been applied to the fabric base and properly dried, a coating of suitable varnish is applied which, combining with the underlying coatings of oil, clay and pigment tends to harden and toughen the composition supported on the textile fabric.

Having thus described my invention, what I claim as new and desire to secure by Letters Patent is—

1. A fabric comprising a textile fabric having a napped surface, a coating of oil applied to the napped surface and dried.

2. A fabric comprising a textile fabric having a cotton base, and a wool napped surface, a coating of oil applied to the napped surface and dried.

3. A fabric comprising a textile fabric of a springy nature, and a coating of oil combined with clay.

4. A fabric comprising a textile fabric of a springy nature, and a coating of oil combined with clay and pigment.

5. A fabric comprising a textile fabric of a springy nature, a series of coatings of oil, clay and pigment applied to the fabric, the outer coatings containing a toughening element.

6. A fabric comprising a textile fabric of a springy nature, a series of coatings of oil, clay and pigment applied to the fabric, the outer coatings containing a toughening element, and a finishing coating of varnish.

In testimony whereof I have signed my name to this specification in the presence of two subscribing witnesses.

CHARLES W. ROYCE.

Witnesses:

ADA E. HAGERTY,  
J. A. MILLER.

Copies of this patent may be obtained for five cents each, by addressing the "Commissioner of Patents, Washington, D. C."